

## UNITED STATES PATENT OFFICE

2,484,456

## METHOD FOR PREPARING PHOTOGRAPHIC EMULSIONS

Wesley G. Lowe and Kearney P. Griffin, Rochester, N. Y., assignors to Eastman Kodak Company, Rochester, N. Y., a corporation of New Jersey

No Drawing. Application March 2, 1946,  
Serial No. 651,610

7 Claims. (Cl. 95—7)

1

This invention relates to non-gelatin silver halide photographic emulsions prepared by peptizing silver halide with polyvinyl pyridine and subsequently mixing the peptized silver halide with a non-gelatin protective colloid for the silver halide.

In the preparation of silver halide photographic emulsions, it is customary to prepare the silver halide in the presence of a peptizing or dispersing agent to obtain a grain size finer than that obtained without the use of the peptizer.

In the preparation of gelatin silver halide emulsions gelatin can be conveniently employed as the peptizing agent, the dispersion formed being readily compatible with further gelatin to form a satisfactory emulsion. Gelatin, however, is incompatible with some of the recognized non-gelatin protective colloids for silver halide. Hydrolyzed gelatin which is more compatible with the protective colloids suffers from the disadvantage that when used as a peptizer for silver halide, emulsion washing causes diffusion of the hydrolyzed gelatin and silver loss occurs. It has been found that the use of polyvinyl pyridine as the peptizer for silver halides has an important advantage over that of gelatin in that polyvinyl pyridine is compatible with non-gelatin protective colloids.

One object of our invention is to provide non-gelatin silver halide emulsions having the degree of speed desired. Another object of our invention is to provide a method of preparing silver halide dispersions which are readily compatible with non-gelatin protective colloids. A further object of our invention is to prepare silver halide dispersions using polyvinyl pyridine as the peptizing agent. Other objects of our invention will appear herein.

Polyvinyl pyridine may be prepared by polymerizing vinyl pyridine, such as by heating to its boiling temperature. A method of preparing polyvinyl pyridine is described in French Patent No. 849,126. The polyvinyl pyridine is dissolved in aqueous acid, such as 1-5% strength acetic acid. Instead of acetic, some other acid may be employed, such as formic, chloracetic, nitric, sulfuric, phosphoric, or the like, the polyvinyl pyridine being most useful in the form of its salt.

After the polyvinyl pyridine is dissolved, silver halide is formed in that solution by introducing a solution of silver salt and a halide into the polyvinyl pyridine solution. This is preferably accomplished by introducing the solutions of halide and silver salt into the polyvinyl pyridine solution simultaneously with agitation or stirring. This

2

dispersion may then be mixed directly with a solution of a non-gelatin protective colloid and sensitized as desired to form a photographic emulsion:

5 The concentration of the solution of polyvinyl pyridine employed to disperse the silver halide is not critical, it only being necessary that sufficient be present to assure dispersion of the silver halide. For instance, as little as  $\frac{1}{2}\%$  will have a peptizing effect, although a considerable formation of silver halide will require more polyvinyl pyridine for best results. A 2% solution of polyvinyl pyridine has been found to be suitable under ordinary conditions of operation. For economic reasons, it is 10 preferable not to exceed a 10% concentration. The amount of acid used need only be sufficient to combine with the polyvinyl pyridine but also in this case, the proportion used is not particularly critical, an excess not interfering with the preparation of the dispersed silver halide.

As the protective colloid or carrier for the dispersed silver halide, any of the non-gelatin materials found to be useful for this purpose may be employed. The far-hydrolyzed cellulose esters as 15 described and claimed in Salo Patent No. 2,110,491, may be employed. Other materials which might be employed are (1) a polyvinyl acetaldehyde having a polyvinyl acetal content of at least 50% and a polyvinyl alcohol content of at least 15% as 20 described and claimed in Fordyce Patent No. 2,211,323; (2) a polyvinyl propionaldehyde or butyraldehyde acetal having a 45-60% vinyl alcohol content in the case of the former, or a 60-80% vinyl alcohol content in the case of the latter as 25 described and claimed in Lowe Patent No. 2,253,078; (3) polyvinyl alcohols (which is the term ordinarily used for compounds which are all polyvinyl alcohol except for 0.5-5% polyvinyl acetate) the use of which in emulsions is disclosed in Lowe Patents Nos. 2,286,215 and 2,276,323, or 30 (4) polyvinyl acetates having a polyvinyl acetate content of 59-71%, the use of which in emulsions is disclosed in the patents referred to in (3).

The following example illustrates our invention:

45 *Example 1.*—Two grams of polyvinyl pyridine were dissolved by stirring with a mixture of 300 cc. of water, 10 cc. of acetic acid and 50 cc. of ethanol. This solution was heated to 84° F. and the following solutions A and B were run therein simultaneously with good stirring over a period of two minutes:

50 *Solution A.*—Ten grams of silver nitrate dissolved in water and made up to a total volume of 20 cc.

*Solution B.*—7.6 grams of potassium bromide and 0.24 gram of potassium iodide dissolved in water and made up to a total volume of 20 cc.

The silver halide formed was very fine grained. The silver halide dispersion was mixed with 100 grams of a 12% aqueous solution of polyvinyl alcohol (viscosity—22 secs.). The mixture was diluted with water to the viscosity desired for smooth coating. The resulting emulsion was sensitized by adding 4 mg. of 2,3'-diethyl-4'-methyloxathiazolocarbocyanine iodide and the coated out onto a baryta-coated paper. It is to be understood that all of the above procedures were carried out under darkened conditions to avoid deterioration of the silver halide.

The photographic paper thus prepared had a low contrast and very low speed and, therefore, could be handled safely in subdued daylight. It developed and fixed readily in the conventional developing and fixing baths.

Our invention includes the preparation of any of the silver halides (Cl, Br, or I) or their mixture. Although our invention has been described in conjunction with the use of non-gelatin protective colloids, the preparation of silver halide dispersions with polyvinyl pyridine for gelatino silver halide photographic emulsions is also within the scope of our invention.

We claim:

1. A silver halide dispersion essentially consisting of a suspension of silver halide prepared by a double decomposition reaction in an aqueous solution of polyvinyl pyridine.

2. A method of preparing a photographic silver halide emulsion which comprises preparing silver halide by double decomposition between a water-soluble silver salt and a water-soluble halide in an aqueous solution of polyvinyl pyridine and subsequently mixing the so-prepared silver halide containing polyvinyl pyridine with a protective colloid therefor.

3. A method of preparing a photographic silver halide emulsion which comprises preparing silver halide by double decomposition between a water-soluble silver salt and a water-soluble halide in

an aqueous solution of polyvinyl pyridine and subsequently mixing the so-prepared silver halide containing polyvinyl pyridine with a non-gelatin protective colloid therefor.

4. A method of preparing a photographic silver halide emulsion which comprises preparing silver halide by double decomposition between a water-soluble silver salt and a water-soluble halide in an aqueous solution of polyvinyl pyridine and subsequently mixing the so-prepared silver halide containing polyvinyl pyridine with polyvinyl alcohol as the protective colloid therefor.

5. A photographic silver-halide emulsion comprising an aqueous mixture of finely dispersed silver halide, polyvinyl pyridine in which the dispersed silver halide was prepared by a double decomposition reaction, and a protective colloid for the dispersed silver halide.

6. A photographic silver-halide emulsion comprising an aqueous mixture of finely dispersed silver halide, polyvinyl pyridine in which the dispersed silver halide was prepared by a double decomposition reaction and polyvinyl alcohol as the protective colloid for the dispersed silver halide.

7. A method of preparing a silver-halide dispersion which comprises simultaneously adding to an aqueous solution of polyvinyl pyridine aqueous solutions of silver nitrate and of alkali metal halides.

WESLEY G. LOWE.  
KEARNEY P. GRIFFIN.

#### REFERENCES CITED

The following references are of record in the file of this patent:

#### UNITED STATES PATENTS

| Number    | Name     | Date          |
|-----------|----------|---------------|
| 2,276,322 | Lowe     | Mar. 17, 1942 |
| 2,281,703 | Lowe     | May 5, 1942   |
| 2,322,085 | Yutzy    | June 15, 1943 |
| 2,397,865 | Jennings | Apr. 2, 1946  |